

Sept. 9, 1924.

1,507,836

C. R. KING

POLISHING WHEEL

Filed July 30, 1921

*Fig. 1*



*Fig. 2*



*Fig. 4*



Witnesses

*John H. McNamee*  
John H. McNamee

Harold W. Eaton

*Fig. 3*

Inventor  
Clarence R. King

By Clayton R. Jenkins  
Attorney

## UNITED STATES PATENT OFFICE.

CLARENCE R. KING, OF WORCESTER, MASSACHUSETTS, ASSIGNEE TO NORTON COMPANY, OF WORCESTER, MASSACHUSETTS, A CORPORATION OF MASSACHUSETTS.

## POLISHING WHEEL.

Application filed July 30, 1921. Serial No. 488,615.

To all whom it may concern:

Be it known that I, CLARENCE R. KING, a citizen of the United States of America, residing at Worcester, in the county of Worcester and State of Massachusetts, have invented certain new and useful Improvements in Polishing Wheels, of which the following is a full, clear, and exact specification.

My invention relates to the abrasive art and more particularly to abrasive wheels for polishing.

The operation of polishing is that by which rough surfaces left after forging, rolling, etc., or scratches and tool marks are removed and a smooth finish secured. The wheels ordinarily utilized for this operation are either wooden wheels covered with leather and turned to fit the piece to be polished or laminated wheels made of sheets of cloth stitched together. In order to make a polishing implement of such a wheel, it is customary to coat the periphery with hot glue and embed therein a layer of abrasive grains of the desired size, this operation of setting up a wheel being laborious, expensive and requiring the services of a skilled operator. When it is considered that set-up wheels of this type may be serviceable for polishing but a very few articles before the abrasive surface must be recoated, it will be seen that it is highly desirable to utilize a wheel which has abrasive throughout a considerable portion of its volume so that it may wear down to a smaller size and still retain its abrading characteristics.

In polishing surfaces of uneven contour, it is essential that the polishing wheel have a slight degree of resiliency in its body so that the outer abrading surface may follow the shape of the article. Hence, the ordinary grinding wheels made of abrasive grains bonded with vitrified clays or similar hard substances are not well adapted for such polishing purposes.

It is accordingly an object of my invention to overcome these difficulties and to provide an economical and serviceable polishing wheel which has a resilient body and is able to conform to a contour and which, unlike the abrasive coated, set-up wheels, has abrasive material throughout a considerable ra-

dial depth and retains its abrading characteristics during repeated use.

With this and other objects in view as will be apparent in the following disclosure, my invention resides in the construction of a polishing wheel as set forth in the specification and covered by the claims appended hereto.

I have illustrated one embodiment of my invention by the accompanying drawings in which:

Figure 1 is a perspective view of a resilient grinding wheel;

Fig. 2 is a detail in perspective of the resilient body of the wheel shown in Fig. 1;

Fig. 3 is a similar view of one of the abrasive strips; and

Fig. 4 is a perspective view, partly broken away, of a modified form of my invention.

I have discovered that the essential requirements are met by an abrasive article having a resilient cushioning body and spaced surface portions or teeth of abrasive material united therewith, which is adapted for polishing. The spaced abrading teeth, in addition to being resiliently supported, are separated by webs of resilient material, to give the desired flexibility and permit the abrading portions to be yieldingly held against the surface being treated. These teeth, which are preferably made of bonded abrasive grains, may be of regular geometrical patterns or irregularly shaped and spaced, the essential feature being that they are so spaced and supported as to be movable with the desired degree of freedom and yet have high polishing or grinding ability. This may be accomplished by mounting or embedding the abrading teeth in a central resilient body made preferably of rubber.

One type of a polishing wheel may be made in accordance with my invention as shown in Figs. 1, 2 and 3. The center portion 10 of the wheel may be made of a resilient material, such as rubber, having radial projections or webs 12 between which are inserted the spaced abrading teeth 14. These teeth may be in the form of parallel strips made from suitably bonded abrasive grains and formed into a unitary structure with the center portion by vulcanization or other

method. A central hole 16 is provided for the subsequent mounting of the wheel upon a spindle conforming with the equipment with which it is to be used.

- 5 For certain purposes, it is preferable that the teeth be of irregular shapes interspersed throughout the resilient body. As shown in Fig. 4, such a wheel may be made of a rigid center 20 provided with a hole 21 and 10 a dovetailed slot 22 in the periphery into which is fitted an abrasive ring 23. In this type of wheel, the resilient body 24, which may be of desired radial thickness, carries the abrasive portions 25 in its outer annular 15 zone or in certain instances distributed throughout its whole volume, as illustrated.

In one method of making a grinding or polishing wheel in accordance with my invention, a mixture is prepared of rubber, a 20 vulcanizing agent such as sulphur and a suitable filler such as barytes or abrasive grains of suitable size, in which the ingredients are thoroughly distributed throughout the mass. A suitable composition which will 25 give the desired degree of resiliency may contain the following materials in the proportions given:

(A) 86.7% filler, 12.6% rubber, 0.7% sulphur.

- 20 This mixture is rolled out into sheets of convenient thickness and cut into the desired shape by means of dies, all of which is common practice in the art. For example, to make a wheel of the type shown in Fig. 25 1, which is a convenient shape for some purposes, disks 10 (Fig. 2) are formed with the radially projecting webs 12 and slots 18 and a hole 16 in the center for the bushing on which it is to be mounted when in use. 40 In order to make a thick wheel, I employ two or more of the thin disks shown in Fig. 2, and place them face to face in the vulcanizing mold, so that they when vulcanized may form a solid body of desired thickness 45 as determined by the number of disks employed.

In like manner, the hard abrasive strips or teeth 14 (Fig. 3) are molded of such size and shape as to fit the slots in the cylinder 50 which has been thus formed. The teeth are formed of abrasive grains bonded with any suitable bond employed in this art. A mixture adapted for this part of the wheel may be composed as follows:

55 (B) 86.7% abrasive grains, 8.9% rubber, 4.4% sulphur.

These strips are inserted into the slots of the body formed of the superimposed disks 10 and the complete wheel then set into a cylindrical mold and subjected to hydraulic pressure by which the various sections are intimately joined together and a smooth cylindrical surface obtained on the outside. While under such pressure it is of course necessary that an iron core be inserted into

the center hole of the wheel to prevent deformation. After pressing, this core is removed and the wheel taken out of the mold and set into a suitable vulcanizer, where it is brought up to a vulcanizing temperature 70 of approximately 300° F. and held at that temperature for about three hours.

In making the modified form of grinding wheel, a mixture is prepared of a suitable resilient material, such as unvulcanized rubber, and small irregular lumps composed of bonded abrasive grains. For the resilient part of this mixture the composition (A) given above may be employed. The abrasive lumps may be made by separately vulcanizing a block molded from the composition (B) and then crushing it to the desired size. The resilient material is then mixed with the vulcanized lumps containing abrasive grains, and the mixture is packed into the 80 mold around the outer edge of the solid center to which it is made to adhere by tamping or pressing into place. The whole wheel thus molded is then subjected to a vulcanization of such a degree as may be necessary 90 for the hardness and rigidity required.

On account of the smaller amount of sulphur contained in the matrix or central portion of the wheel, this part will be relatively soft and resilient or elastic. The 95 abrasive portion, which contains a larger amount of sulphur, even though it has been subjected to the same vulcanizing treatment, as in the first case, will be considerably harder and more rigid. Moreover, being 100 thus vulcanized in intimate contact with each other, the sections will have been joined firmly by the webs of resilient rubber and will present a unitary structure. Accordingly, when the wheel is mounted upon an 105 arbor and rotated with its surface in contact with an article to be ground, the grinding action of each abrasive tooth, as it comes in contact with the work, will be essentially that of an abrasive article having the hardness of the outer surface. It will not make a rigid contact with the work, however, on account of the soft or elastic backing, which will permit it to yield to the pressure of contact and thus prevent the deep cutting action 110 which a wheel, having the hardness of the abrasive portions throughout, would give. At the same time the outer surface will possess sufficient rigidity to give the desired 115 grinding action and produce a highly polished surface.

While I have specifically described my invention as adapted to the manufacture of an abrasive wheel of a rubber composition, it will be obvious to those skilled in the art 125 that other abrasive articles in which the same or similar properties are desired may be as readily made, and that other materials and other proportions may also be used to suit the particular conditions which may in 130

any case be involved. Such modifications or substitutions of my invention are, however, to be considered as embodied in the above specification and in the following 5 claims.

I claim:

1. An abrasive article comprising a resilient cushioning body and spaced teeth of bonded abrasive grains united therewith.
- 10 2. An abrasive article comprising a body, a plurality of spaced portions of rubber bonded abrasive grains, and resilient rubber webs separating and supporting the bonded abrasive portions on said body.
- 15 3. An abrasive wheel comprising a resili-

ent cushioning body of rubber and a plurality of spaced teeth of bonded abrasive grains united and having a continuous surface with said body.

4. An abrasive wheel comprising a resilient rubber center portion, a plurality of spaced teeth of rubber bonded abrasive grains supported thereby, and webs of resilient rubber separating and uniting the teeth with said center portion, said webs and teeth having a common continuous surface.

Signed at Worcester, Massachusetts, this 21st day of July, 1921.

CLARENCE R. KING.